

1

3,782,907

**IRIDESCENT CHROMIUM PLATED ARTICLE**  
Hyman Chessin, 7146 Heather Heath Lane, Birmingham,  
Mich. 48010, and Robert Francis Gempel, 71 W.  
Hancock, Apt. 3, Detroit, Mich. 48201  
No Drawing. Original application Feb. 6, 1969, Ser. No.  
797,258, now Patent No. 3,657,079. Divided and this  
application May 6, 1971, Ser. No. 141,044  
Int. Cl. B32b 15/00

U.S. Cl. 29—194

3 Claims

### ABSTRACT OF THE DISCLOSURE

This invention relates to novel compositions and to a process of preparing an iridescent chromium plated article which comprises passing current from an anode to a cathode through an aqueous chromium plating solution which contains at least one chromium compound providing chromium metal ions for electroplating chromium and a hexavalent molybdenum compound to produce an iridescent chromium surface on said cathodic article.

This application is a divisional application of Ser. No. 797,258, filed on Feb. 6, 1969, now U.S. Pat. No. 3,657,079.

This invention relates to a novel decorative metal coating, to bath compositions used to prepare such coatings, and to processes for the preparation of such metal coatings. More particularly, this invention relates to decorative electrodeposited chromium surfaces which have iridescent properties.

According to one aspect of the invention, a bath containing a hexavalent chromium compound and a hexavalent molybdenum compound is employed to produce an electroplated article with a chromium metal surface which reflects light to give an iridescent, rainbow effect.

The aqueous chromium plating solution employed according to the invention may be prepared from commercial chromic acid solutions. Preferably, a portion of the chromic acid used in the bath composition may be replaced by a salt of hexavalent chromium such as sodium chromate, sodium dichromate, potassium chromate, potassium dichromate, strontium chromate, magnesium dichromate, lanthanum chromate, lanthanum dichromate, etc. In many cases it may be advantageous to employ one or more of such salts in order to provide for a means of control of the composition or of the acidity of the aqueous chromium plating bath.

Any molybdenum compound soluble in the bath composition which yields hexavalent molybdenum may be employed as a component of the aqueous chromium plating bath composition to provide a chromium plated article having iridescent properties. Molybdcic acid is a highly preferred component which may be employed in the bath composition. Typically, molybdcic acid may be used as an ammonium complex of molybdcic oxide containing about 8.5% by weight of ammonium ion and about 85% by weight molybdcic oxide. Other typical hexavalent molybdenum compounds which may be used include sodium molybdate, phosphomolybdcic acid, etc.

Catalyst anions may also be included in the aqueous chromium plating bath to regulate the concentrations of the active ingredients during electroplating. For example, sulfate, fluoride, and complex fluorides may be used.

2

Typically, fluosilicates, fluoborates, fluoaluminates, fluotitanates, and fluozirconates may be included in the aqueous chromium plating bath composition without adversely affecting the iridescent light reflective properties of the novel decorative chromium electroplate which is produced according to the invention.

Suitable neutralizers and/or buffers may also be employed in the bath composition of the invention. Examples of such neutralizers or buffers may include phosphates, borates, sulfonates, and carboxylates. In addition, catalyst anions as heretofore recited may also be used in amounts sufficient to act as buffers or neutralizers in combined effect with their catalyst properties.

A typical bath composition which may be used according to the process of the invention to produce an iridescent chromium electrodeposit may comprise chromic acid in an amount of 50–600 g./l. as  $\text{CrO}_3$  in combination with a hexavalent molybdenum compound in an amount of 2–140 g./l. as  $\text{MoO}_3$ . Other adjuvant materials may be included in the bath.

A specific bath composition may contain the following ingredients in the amounts indicated:

|                                 |        |     |
|---------------------------------|--------|-----|
| Chromic acid                    | g./l.  | 300 |
| Sulfate                         | g./l.  | 1.2 |
| Molybdcic acid (85% by weight)  | g./l.  | 110 |
| Concentrated ammonium hydroxide | ml./l. | 20  |

When a sulfate catalyst anion is employed as a component of the iridescent chromium plating bath composition, the amount of sulfate anion may typically be 0.3–3.0 g./l. Other typical ranges for preferred catalyst anions and buffer include:

TABLE I

|                | G./l.    |
|----------------|----------|
| Fluoride       | 0.1–1.0  |
| Silicofluoride | 0.5–5.0  |
| Phosphate      | 0.35–3.5 |
| Acetate        | 2.0–20   |

The catalyst and/or buffer anions may be employed individually or in any combination wherein the combined amounts of said catalyst anions may be 0.3–30 g./l. based upon the weight of the total bath composition.

Other typical materials which yield regulating buffer ions include trichloroacetic acid, succinic anhydride, adipic acid, and sodium aluminate. Said ingredients may be used in the iridescent chromium plating bath compositions of the invention in amounts (based upon the total weight of the composition) of 0–40 g./l.

In an iridescent chromium plating bath employed according to the invention, the ratio of chromic acid ( $\text{CrO}_3$ ) to (calculated) molybdenum trioxide ( $\text{MoO}_3$ ) may be from 3:1–40:1. Thus, for an aqueous iridescent chromium plating bath which may contain 250 g./l. chromic acid ( $\text{CrO}_3$ ) the bath composition may contain 40–70 g./l. of molybdcic acid ( $\text{MoO}_3$ ). Amounts of chromic acid as  $\text{CrO}_3$  of from 50–600 g./l. may be used and, preferably, baths containing 225–275 g./l. of chromium and 30–80 g./l. of molybdcic acid as  $\text{MoO}_3$  are employed.

The iridescent chromium plated articles prepared using the compositions of the invention may contain mounds of chromium deposits having a mean height above the surface of 0.025–5 microns wherein said mounds are posi-

tioned in adjacent and semi-overlapping strings, said strings being positioned in approximately parallel configurations to form an iridescent chromium surface having from 70-1500 strings per millimeter and  $6 \times 10^5$ - $6 \times 10^8$  mounds of chromium deposits per square centimeter of surface. Such iridescent chromium plated articles may be subsequently given a supplementary metallic coating of metals such as nickel, copper, chromium, etc. to enhance or modify the color or reflectivity of the iridescent surface. Similarly, organic or inorganic coatings may be used to vary the decorative rainbow effects on all or a portion of said surfaces.

The mounds of chromium deposits are roughly circular in cross section and may have a curvature approaching that of a sphere or a portion of a sphere. The mean height of a mound of chromium deposit is measured from the plane which joins the totality of points representing the average of the minimum and maximum of the surface upon which said mounds are positioned. Microscopic examination of said surface shows that the mounds of deposit may be completely separate with distances between said mounds of up to three or four mound diameters. The mounds may touch or overlap to form continuous strings or semi-continuous strings, said strings being positioned in approximately parallel configurations analogous to strings of beads placed upon and conforming the shape of a given surface. It is believed that the parallel configurations (which are not necessarily linear) produce an effect such as may be obtained from a diffraction grating using parallel lines. It has been found that particularly striking iridescent effects may be obtained from an iridescent chromium plated article wherein the article contains about  $6 \times 10^5$ - $6 \times 10^8$  mounds having an average height of 0.025-5 microns, wherein the mounds are positioned on the surface of said iridescent chromium plated article so that a series of continuous lines connecting the centers of said mounds produces a network of lines and said network of lines contains at least 790 parallel lines per linear centimeter of length as measured by intersecting points on a straight line drawn in any direction for a length of one centimeter from the center of a given mound of iridescent chromium plated surface. Thus, a line of one centimeter length drawn from any given mound on the chromium plated surface of the iridescent chromium plated article of the invention intersects at least about 790 approximately parallel strings of mounds when such strings of mounds are connected by lines drawn to the centers of the mounds comprising said approximately parallel strings.

Bright iridescent chromium plated articles may be characterized as having a surface containing mounds of chromium deposits wherein the average height of the mounds is about 0.075-2.5 microns and wherein the average space between any two approximately parallel adjacent strings of mounds (as measured by the average distance between the two lines joining the center of each of the mounds of each string) is about 2.5 microns. Particularly brilliant iridescent chromium plated surfaces may be obtained when the average height of the mounds is about 0.087 micron and the average space between any two approximately parallel adjacent strings of mounds (as measured by the average distance between two lines joining the center of the mounds of each string) is approximately 2.9-3.0 microns.

The following examples are submitted for the purpose of illustration only and are not to be construed as limiting the scope of the invention in any way.

#### EXAMPLE 1

An iridescent chromium plating bath composition was prepared by combining the following ingredients in water with the indicated concentrations (all concentrations being in grams per liter of total solution unless otherwise specified herein):

|                                                | Grams per liter (g./l.) |
|------------------------------------------------|-------------------------|
| Chromic acid ( $\text{CrO}_3$ )                | 250                     |
| Molybdic acid (85%)                            | 50                      |
| Fluoride ( $\text{F}^-$ )                      | 0.3                     |
| Sulfate ( $\text{SO}_4^{=2-}$ )                | 1.0                     |
| Acetate ( $\text{C}_2\text{H}_3\text{O}_2^-$ ) | 10.4                    |
| Phosphate ( $\text{PO}_4^{=3-}$ )              | 0.1                     |

A steel strip was chromium plated in the above iridescent chromium plating solution by passing plating current through said bath composition using the metal strip as electrode for five minutes at a temperature of 40°-45° C. The chromium plated article was removed from the bath, rinsed, dried, and was noted to display an iridescent effect when exposed to sunlight and artificial light.

#### EXAMPLE 2

Example 1 was repeated using a nickel-plated steel strip as electrode in the iridescent chromium plating bath composition of Example 1 at a temperature of 49° C. with a plating time of 15 minutes and a plating current density of approximately 20 a.s.d. (amperes per square decimeter). The chromium plated article obtained was noted to produce iridescent effects when exposed to sunlight and artificial light. Similar iridescent surfaces were obtained using a plating time of one minute to produce the chromium electrodeposits.

#### EXAMPLE 3

An iridescent chromium plating bath composition was prepared by combining the following ingredients in the indicated concentrations in water:

|                                                | Grams per liter (g./l.) |
|------------------------------------------------|-------------------------|
| Chromic acid ( $\text{CrO}_3$ )                | 300                     |
| Molybdic acid (85% $\text{MoO}_3$ )            | 60                      |
| Sulfate ( $\text{SO}_4^{=2-}$ )                | 1.2                     |
| Fluoride ( $\text{F}^-$ )                      | 0.4                     |
| Phosphate ( $\text{PO}_4^{=3-}$ )              | 0.6                     |
| Acetate ( $\text{C}_2\text{H}_3\text{O}_2^-$ ) | 15-17                   |

A die-cast automobile door handle was connected as electrode and immersed in the above iridescent chromium electroplating composition. Electroplating current was passed through the article to be electroplated and the solution at a temperature of about 44° C. to obtain an iridescent chromium electroplate on the die-cast automobile door handle.

#### EXAMPLE 4

An iridescent chromium plating bath composition was prepared by combining the following ingredients in the indicated concentrations in water:

|                                                | Grams per liter (g./l.) |
|------------------------------------------------|-------------------------|
| Chromic acid ( $\text{CrO}_3$ )                | 250                     |
| Molybdic acid (85% $\text{MoO}_3$ )            | 50                      |
| Sulfate ( $\text{SO}_4^{=2-}$ )                | 1.0                     |
| Fluoride ( $\text{F}^-$ )                      | 0.3                     |
| Phosphate ( $\text{PO}_4^{=3-}$ )              | 0.4                     |
| Acetate ( $\text{C}_2\text{H}_3\text{O}_2^-$ ) | 14                      |

A copper plated strip was connected as electrode, immersed in the above iridescent chromium plating composition and current was passed through said solution at about 44° C. to produce an iridescent chromium electrodeposit on said copper strip.

The following Examples 5-20 were carried out in a Hull cell in order to demonstrate that iridescent chromium deposits may be produced according to the process of the invention over wide current density ranges. The concentrations (in grams per liter unless specified otherwise) are given for each ingredient in the aqueous iridescent chromium plating bath and the results and conditions are summarized in Table II. In each example a standard plating time of five minutes was used and the temperature was maintained at 43°-44° C. for purposes of comparison.

The total length of the standard Hull cell used in the experiments was 100 millimeters.

positions wherein the average height of the chromium mounds is about 0.075-2.5 microns and said mounds are

TABLE II

| Example number | Ingredient concentration (g./l.) |                  |                 |                 |                                              |                                      | Standard hull cell current (amps) | Length of hull cell iridescent span (mm.) | Remarks    |
|----------------|----------------------------------|------------------|-----------------|-----------------|----------------------------------------------|--------------------------------------|-----------------------------------|-------------------------------------------|------------|
|                | CrO <sub>3</sub>                 | MoO <sub>3</sub> | SO <sub>4</sub> | PO <sub>4</sub> | C <sub>2</sub> H <sub>3</sub> O <sub>2</sub> | Other                                |                                   |                                           |            |
| 5              | 500                              | 140              | 2.5             | 0               | 0                                            | Na <sub>2</sub> O (60)               | 12                                | 53                                        | Excellent. |
| 6              | 400                              | 119              | 2.0             | 0               | 0                                            | Na <sub>2</sub> O (51)               | 12                                | 45                                        | Do.        |
| 7              | 250                              | 42.5             | 0.9             | 0.7             | 15.6                                         | F <sup>-</sup> (0.3)                 | 8                                 | 60                                        | Superior.  |
| 8              | 128                              | 21.8             | 0.46            | 0.36            | 9.7                                          | ZrF <sub>6</sub> <sup>-</sup> (0.31) | 8                                 | 56                                        | Do.        |
| 9              | 80                               | 8.5              | 0.29            | 0.22            | 10.6                                         | F <sup>-</sup> (0.10)                | 8                                 | 58                                        | Do.        |
| 10             | 300                              | 50               | 0               | 0.42            | 18                                           | SiF <sub>6</sub> <sup>-</sup> (6.0)  | 8                                 | 68                                        | Do.        |
| 11             | 300                              | 60               | 1.2             | 0               | 0                                            | CaCO <sub>3</sub> (40-55)            | 8                                 | 50                                        | Excellent. |
| 12             | 250                              | 50               | 0.9             | 0.7             | 15.6                                         | F <sup>-</sup> (0.3)                 | 8                                 | 70                                        | Superior.  |
| 13             | 200                              | 45               | 0.8             | 0               | 0                                            | Na <sub>2</sub> O (7.6)              | 8                                 | 52                                        | Excellent. |
| 14             | 300                              | 60               | 1.1             | 0.7             | 0                                            | 0                                    | 8                                 | 45                                        | Do.        |
| 15             | 250                              | 42.5             | 0.9             | 0.7             | 15.6                                         | SiF <sub>6</sub> <sup>-</sup> (0.9)  | 8                                 | 60                                        | Superior.  |
| 16             | 250                              | 42.5             | 0.9             | 0.7             | 15.6                                         | TiF <sub>6</sub> <sup>-</sup> (0.75) | 8                                 | 62                                        | Do.        |
| 17             | 250                              | 42.5             | 0.9             | 0.7             | 15.6                                         | ZrF <sub>6</sub> <sup>-</sup> (0.6)  | 8                                 | 61                                        | Do.        |
| 18             | 250                              | 42.5             | 0.6             | 0.7             | 15.6                                         | AlF <sub>6</sub> <sup>-</sup> (1.2)  | 8                                 | 59                                        | Do.        |
| 19 (standard)  | 250                              | 0                | 0.6             | 0.7             | 15.6                                         | SiF <sub>6</sub> <sup>-</sup> (0.9)  | 8                                 | 0                                         |            |
| 20 (standard)  | 250                              | 0                | 1.0             | 0.4             | 14.6                                         | F <sup>-</sup> (0.3)                 | 12                                | 0                                         | { (*)      |

<sup>1</sup> Ordinary chromium plate—no iridescent effects.

As can readily be seen from Table II excellent or superior results were obtained using the compositions set forth in Examples 518, whereas an ordinary chromium plate was obtained in Examples 19 and 20 (denoted as standards) when hexavalent molybdenum was omitted from the bath compositions. In Table II a Hull cell containing an iridescent span of at least 40 millimeters of continuous length of the Hull cell is considered to have an "excellent" rating, whereas continuous iridescent spans of over 55 millimeters in length are considered "superior." In each case the iridescent effect was compared both in natural sunlight and in artificial light including incandescent and fluorescent light.

Although this invention has been illustrated by reference to specific embodiments, modifications thereof which are clearly within the scope of the invention will be apparent to those skilled in the art.

What is claimed is:

1. An iridescent chromium plated article wherein the surface of the article contains about  $6 \times 10^5$ - $6 \times 10^8$  mounds of chromium deposit per square centimeter, said mounds having an average height of 0.025-5 microns and positioned on the surface of said iridescent chromium plated article so that a series of continuous lines connecting said mounds produces a network of lines wherein said network of lines contains at least about 790 parallel lines per linear centimeter of length as measured by intersecting points of a straight line drawn in any direction for a length of one centimeter from the center of a given mound of iridescent chromium plated surface.

2. An iridescent chromium plated article wherein the chromium surface contains mounds of chromium de-

positioned in adjacent and semi-overlapping strings, said strings being positioned in approximately parallel configurations to form a surface having about 70-1500 strings per millimeter and wherein the average space between any two approximately parallel adjacent strings of mounds as measured by the distance between the two lines joining the centers of the mounds of each string is about 2.5 microns.

3. An iridescent chromium plated article wherein the chromium surface contains mounds of chromium deposits wherein the average height of the chromium mounds is about 0.087 micron and said mounds are positioned in adjacent and semi-overlapping strings, said strings being positioned in approximately parallel configurations to form a surface having about 70-1500 strings per millimeter and wherein the average space between any two approximately parallel adjacent strings of mounds is 2.9-3.0 microns.

#### References Cited

##### UNITED STATES PATENTS

|           |         |              |          |
|-----------|---------|--------------|----------|
| 3,113,845 | 12/1963 | Uchida       | 29—196.6 |
| 3,157,585 | 11/1964 | Durham       | 29—196.6 |
| 3,418,221 | 12/1968 | Woods        | 204—51   |
| 3,428,441 | 2/1969  | Du Rose      | 29—196.6 |
| 3,461,048 | 8/1969  | Mahlstedt    | 204—51   |
| 2,412,698 | 12/1946 | Vander Horst | 29—196.6 |

HYLAND BIZOT, Primary Examiner

U.S. Cl. X.R.

29—196.6